

C. Mc BURNEY.  
STRAP FOR DROP PRESSES.

No. 40,349.

Patented Oct. 20, 1863.

Fig 1



Fig 2



Netnesses  
J. C. Vaughan  
D. C. Fidchemacher

Inventor  
Chas McBurney  
By his attorney  
Sam Cooper

# UNITED STATES PATENT OFFICE.

CHARLES McBURNEY, OF ROXBURY, MASSACHUSETTS.

## IMPROVED STRAP FOR DROP-PRESSES.

Specification forming part of Letters Patent No. 40,349, dated October 20, 1863.

*To all whom it may concern:*

Be it known that I, CHARLES McBURNEY, of Roxbury, in the county of Norfolk and State of Massachusetts, have invented certain improvements in the manufacture of straps for drop-presSES, which are also applicable to the manufacture of machine-beltiNG, of which the following is a full, clear, and exact description, reference being had to the accompanying drawings, making part of this specification, in which—

Figure 1 represents the canvas employed, showing the lines upon which it is cut up. Fig. 2 illustrates the manner in which the canvas is folded in making my improved strap.

Straps for drop-presSES have usually been made of two or more thicknesses of leather sewed or riveted together. After use for a short time these straps become exceedingly hard and rigid and lose the little elasticity which they originally possess. They are then liable to break at the instant when the power is applied to elevate the weight, besides which they are originally very expensive.

My invention has for its object to produce a strap that shall possess a limited degree of elasticity, or such a capability of yielding on the application of the power to elevate the weight as to prevent the effect of the sudden application of force to the strap; and my invention consists of a belt or strap formed of successive layers of canvas cut diagonally across the piece and folded so as to bring both the warp and the weft threads diagonal to the length of the strap, that the strain at no point may come directly upon the threads or in the direction of their length.

In the manufacture of my improved semi-elastic strap I employ canvas, duck, or any suitable woven goods having the requisite strength, which is coated upon both sides with the rubber compound in the ordinary way, so that the weight of the compound shall be about equal to that of the cloth. It is then cut diagonally upon the lines *a a*, Fig. 1, and the strap is formed by folding over and over successive plies of the material, the folds being made parallel to the lines *a a*, Fig. 2, so as to bring the threads of the warp and weft diagonal to the strap in the direction of its length. The strap is then confined between metallic plates and vulcanized by heating in any well-known manner.

A strap thus made is found to possess a strength far surpassing that of a leather strap or of one of canvas in which the folds are made parallel with the warp-threads, for two principal reasons—first, on account of its superior elasticity, which enables the strain to which it is subjected to be put upon it gradually; secondly, on account of the increased number of threads which assist to bear the strain.

In a rigid, non-elastic strap, as in the case of one made of leather or of india-rubber and canvas put together in the ordinary way—that is, with the folds parallel with the warp-threads—as all the strain is applied by a sudden jerk or twitch, and as the weight amounts oftentimes to several tons, this strain is immense. Where, on the other hand, the threads of the canvas run diagonally, the strip, in lieu of being rigid, is rendered so elastic that the weight is thrown upon it very gradually, and the strap is therefore submitted to a far less strain. At the same time that this is the case, the strap is also intrinsically much stronger, for while in the one case the warp-threads alone sustain the weight, in the other both the warp and the weft threads unite to give strength to the strap. The original cost of this strap is also far less than that of the ordinary leather strap.

The compound which I prefer for the manufacture of my improved strap is made as follows: twenty-five pounds crude rubber, ten pounds white lead, and two pounds sulphur, the whole being ground together upon the ordinary heated rolls and spread upon the canvas in the well-known manner.

I do not, however, confine myself to any particular compound or to any exact proportions of the ingredients, as these may be varied to a considerable extent without materially affecting the result.

What I claim as my invention, and desire to secure by Letters Patent, is—

The improved strap or belt for drop-presSES, composed of several plies of canvas cut diagonally and cemented together with vulcanized india-rubber, as set forth.

CHARLES McBURNEY.

Witnesses:

SAM. COOPER,  
P. E. TESCHEMACHER.